

S. P. BUSH.

METHOD OF MAKING CAR WHEELS.

APPLICATION FILED APR. 13, 1912.

1,047,379.

Patented Dec. 17, 1912.



WITNESSES

*E. J. Birmingham*  
*G. J. Downing*

INVENTOR

*S. P. Bush*  
*By H. G. Seymour*  
*Attorney*

# UNITED STATES PATENT OFFICE.

SAMUEL P. BUSH, OF COLUMBUS, OHIO.

## METHOD OF MAKING CAR-WHEELS.

1,047,379.

Specification of Letters Patent. Patented Dec. 17, 1912.

Application filed April 13, 1912. Serial No. 690,653.

To all whom it may concern:

Be it known that I, SAMUEL P. BUSH, a citizen of the United States, residing at Columbus, in the county of Franklin and State of Ohio, have invented certain new and useful Improvements in Methods of Making Car-Wheels; and I do hereby declare the following to be a full, clear, and exact description of the invention, such as will enable others skilled in the art to which it appertains to make and use the same.

My invention relates to an improvement in the method of making car wheels having a rim portion of one kind of metal, and a central or inner portion of another kind, both kinds of metals being specially adapted for the purpose of the service intended, and is designed particularly as an improvement on the invention disclosed in my allowed application filed March 21st, 1911, Serial Number 616,006.

It is very desirable in car wheels, to have the rim portion which is subjected to severe usage, of hard, tough, and finely grained steel- or iron alloy, and the hub portion which requires machining to properly fit it to the axle, of softer and more malleable metal, and the object of this invention is to provide means whereby the metal to form the surface of the rim of the wheel will be solidified quickly, and thus prevent it from being displaced by the softer and subsequently poured metal.

My invention consists in pouring the metal for the rim of a steel wheel against a chill whereby the fluid metal will be quickly solidified, and subsequently and without any material delay, pouring the metal for the web and hub, which uniting with the partly solidified rim forms an integral structure.

In the accompanying drawings, Figure 1 is a view of a mold showing the cast wheel thereon. Fig. 2 is a view of the wheel as it leaves the mold and Fig. 3 is a view of the wheel after its hub has been forced into its final position.

1 and 2 represent the two parts of a mold, 3 the hub core, and 4 a chill, the latter adapted to cover that part of the rim of the wheel which is subjected to wear by contact with the rail. The pattern has its hub elevated, above normal and its web inclining downwardly from a point adjacent the upper end of the hub to the rim, so as to produce a wheel as shown in Fig. 2, in which the hub 5 is raised so as to bring its lower

edge approximately in the plane of the flange of the rim 6, and the opposite or upper end of the hub in a plane above the opposite or upper side of the rim. The web 6 connecting the hub 5 and rim 6 is downwardly inclined from the hub outwardly, so that the first metal entering the mold will gravitate down the web section thereof into the rim section, and come into immediate contact with the chill 4. This chill acting on the steel, does not change the physical characteristics of the latter as it does with cast iron, but simply operates to solidify the steel in contact therewith, and for some distance back, so that the subsequent or second metal for the hub and web portion, closely following the first cannot displace the metal already within the rim, and which as previously explained has been more or less solidified by its contact with the chill.

In pouring, the metal is introduced at the center through the hub core, and passes up through the hub into the web and then down into the rim. When sufficient metal has been poured to approximately fill the rim, the pouring is discontinued, and the metal adapted for the hub and web is then poured without any material delay between the two pouring steps. The metal last poured mixes to a certain extent with that in the hub portion of the wheel and forces that within the web 7, into the rim until the latter is filled. As the metal in the rim contacts with the chill it immediately hardens or solidifies to such an extent that it cannot be dislodged or displaced by that following, hence it will be evident that the metal first poured will precede the metal of the second pouring to the rim, and after the first pouring has been discontinued, the metal then in the rim will have solidified to such an extent that it cannot be displaced by any metal subsequently entering the rim.

After the wheel has been cast, and preferably while it is at a forging temperature, I subject the hub and web to pressure between dies or platens to force the hub and web into their proper positions relative to the rim, or into the position shown in Fig. 3. This change in position of the hub relative to the rim shortens up the web between the hub and the rim and operates to relieve internal stress due to shrinkage of the parts.

It is evident that many slight changes might be resorted to in the relative arrangement of parts shown and described without

departing from the spirit and scope of my invention. Hence I would have it understood that I do not wish to confine myself to the exact construction and arrangement of parts shown and described, but

Having fully described my invention what I claim as new and desire to secure by Letters-Patent, is:—

- 10 1. The method of making wheels consisting in providing a mold with a chill section conforming to the rim of the wheel, filling the rim portion of the mold first with a metal which coming in contact with the chill solidifies sufficiently to prevent it from being dislodged by the metal for the hub and rim, and immediately filling the web and hub with a softer metal which unites with the metal in the rim.
- 20 2. The method of making car wheels consisting in forming a mold in which the hub and web portions are elevated above the final position so as to give a downward inclination to the web from the hub to the rim, providing the rim section of the mold with a chill whereby the metal first coming in contact with same will be solidified suffi-

ciently to prevent it from being dislodged by the metal following same, and subsequently forcing the hub and web portions of the wheel into final position.

3. The method of making wheels consisting in providing a mold with a chill section conforming to the rim of the wheel, and with a hub and web section elevated sufficiently to cause the first metal entering the mold through the hub, to pass down into and through the web into the rim and in contact with the chill whereby the metal first poured will be solidified by its contact with the chill sufficiently to prevent it from being dislodged by the metal for the web and hub, and immediately filling the web and hub with a softer metal which unites with the metal in the rim.

In testimony whereof, I have signed this specification in the presence of two subscribing witnesses.

SAMUEL P. BUSH.

Witnesses:

ARNO EBERLEIN,  
GEO. G. MERRING.

---

Copies of this patent may be obtained for five cents each, by addressing the "Commissioner of Patents, Washington, D. C."

---